# EUROPEAN PATENT SPECIFICATION

(11) **EP 1 420 078 B1**
(45) Date of publication and mention of the grant of the patent: **27.02.2019**
(21) Application number: 03026063.2
(22) Date of filing: 12.11.2003
(51) Int. Cl.: C22C 38/44, C22C 38/02, C22C 38/04, C22C 38/50, C22C 38/06, C22C 38/00, C22C 38/46, C22C 38/48, C23C 8/32, C23C 8/22

(54) **Bearing steel excellent in corrosion resistance**
Lagerstahl mit guter Korrosionsbeständigkeit
Acier pour roulements ayant une excellente résistance à la corrosion

(30) Priority: 12.11.2002 JP 2002328854
(43) Date of publication of application: 19.05.2004
(73) Proprietor: JTEKT Corporation, Osaka-shi Osaka 542-8502 (JP)
(72) Inventor: Toshiva, Kinami, Koyo Seiko Co., Ldt., Osaka 542-0081 (JP); Toshimitsu, Kimura, Daido Tokushuko K.K., Aichi (JP); Hisato, Nishisaka, Koyo Seiko Co., Ldt., Osaka 542-0081 (JP); Masao, Goto, Koyo Seiko Co., Ldt., Osaka 542-0081 (JP)
(74) Representative: Grünecker Patent- und Rechtsanwälte PartG mbB

(56) References cited:
- EP-A- 0 763 606
- EP-A- 0 933 440
- GB-A- 763 398
- US-A- 4 026 727
- US-A- 5 383 768
- US-A- 5 595 610
- PATENT ABSTRACTS OF JAPAN vol. 015, no. 285 (C-0851), 19 July 1991 (1991-07-19) -& JP 03 100142 A (KOBE STEEL LTD), 25 April 1991 (1991-04-25)
- PATENT ABSTRACTS OF JAPAN vol. 1995, no. 01, 28 February 1995 (1995-02-28) -& JP 06 287711 A (SUMITOMO METAL IND LTD), 11 October 1994 (1994-10-11)
- PATENT ABSTRACTS OF JAPAN vol. 1996, no. 09, 30 September 1996 (1996-09-30) -& JP 08 120438 A (KOBE STEEL LTD), 14 May 1996 (1996-05-14)
- PATENT ABSTRACTS OF JAPAN vol. 2000, no. 05, 14 September 2000 (2000-09-14) -& JP 2000 054069 A (NIPPON STEEL CORP), 22 February 2000 (2000-02-22)
- PATENT ABSTRACTS OF JAPAN vol. 2000, no. 20, 10 July 2001 (2001-07-10) -& JP 2001 073067 A (SANYO SPECIAL STEEL CO LTD), 21 March 2001 (2001-03-21)
- PATENT ABSTRACTS OF JAPAN vol. 1996, no. 07, 31 July 1996 (1996-07-31) -& JP 08 060294 A (KOBE STEEL LTD), 5 March 1996 (1996-03-05)
- PATENT ABSTRACTS OF JAPAN vol. 018, no. 328 (C-1215), 22 June 1994 (1994-06-22) -& JP 06 073492 A (AICHI STEEL WORKS LTD), 15 March 1994 (1994-03-15)

## Description

### BACKGROUND OF THE INVENTION

The present invention relates to bearing steel and particularly to bearing steel which is excellent in corrosion resistance, surface fatigue strength and rolling fatigue life and which is adapted for large-size bearing parts in a rolling machine (mill), a thermal power generator, a hydraulic powder generator, etc.

A carburized material of case-hardened steel such as JIS SCr, JIS SCM or JIS SNCM has been heretofore used as bearing steel for large-size bearing parts.

There has been however an increasing demand for long-lived bearing parts in recent years. Under such circumstances, attempt to add alloy elements such as Si, Ni, Mo, etc. to thereby improve rolling fatigue strength has been made.

A bearing steel according to the preamble of claim 1 is known from any of JP 03 100142 A, EP 0 933 440 A1, JP 06 287711 A, EP 0 763 606 A1, JP 08 120438 A, JP 2000 054069 A, JP 2001 073067 A, US 5,595,610, US 4,026,727, JP 08 060294 A, GB 763,398 A, JP 06 073492 A and US 5,383,768 A. The therefrom known bearing steel is substantially obtained by a method comprising a heat treatment performed by carburizing followed by quenching and tempering.

For example, Japanese Patent Publication 14416/1990 has disclosed bearing steel adapted for large-size bearing parts and containing JIS SNCM 815 as a base material, and an appropriate amount of Si and Ni added to the base material.

Incidentally, for example, in the case of bearing parts used in a rolling machine, rust may be formed due to penetration of rolling water in accordance with the rolling machine. There is a problem that the rust brings about reduction in rolling fatigue life.

Therefore, development of bearing steel more excellent in corrosion resistance is required newly so that the bearing steel can be adapted for large-size bearing parts.

### SUMMARY OF THE INVENTION

The invention is developed to solve the problem and an object of the invention is to provide bearing steel which is excellent in corrosion resistance, surface fatigue strength and rolling fatigue life.

In order to solve the aforesaid object, a beaving steel according to claim 1 is proposed. Preferred embodiments of the inventive beaving steel ave subject to the dependent claims.

### BRIEF DESCRIPTION OF THE DRAWING

FIG. 1 is a view typically showing rod-like carbide existing in steel.

### DETAILED DESCRIPTION OF PREFERRED EMBODIMENTS

### Operation of the Invention

The inventors have examined various alloy elements. As a result, it has been found that both reduction in the amount of added Si and addition of an appropriate amount of Ni and Cr are effective in improving corrosion resistance.

It has been also apparent that the surface C concentration, the area percentage of carbide and the presence of rod-like carbide after carburizing treatment have large influence on corrosion resistance and rolling fatigue life.

That is, it has been apparent that a surface C concentration high enough to be not lower than a certain degree is required for improving rolling fatigue life but increase in C concentration causes increase in area percentage of carbide to thereby deteriorate corrosion resistance and causes production of rod-like carbide to thereby deteriorate both rolling fatigue life and impact resistance remarkably.

The reason why the presence of rod-like carbide deteriorates both rolling fatigue life and impact resistance can be conceived as follows. That is, the bearing steel cracks along a surface of rod-like carbide which is an inclusion, or the rod-like carbide is apt to operate as a start point of the crack.

It is further conceived that corrosion resistance also deteriorates because the bearing steel is apt to corrode along the surface of the rod-like carbide.

In the invention, it has been found that those properties deteriorate particularly when rod-like carbide having an aspect ratio of not lower than 3 and having a minor diameter of not larger than 2 µm is produced.

The inventors have also found that addition of an appropriate amount of Ni and Mo is effective in improving rolling fatigue life.

The invention is based on the aforementioned knowledge.

In the invention, the size of each oxide inclusion in the steel before carburizing treatment is selected to be not larger than 50 µm in terms of the maximum diameter. That is, the inventors have found that corrosion resistance can be improved when the size of each oxide inclusion in the steel is reduced to be not larger than 50 µm.

It has become also apparent that evaluation of acid-dissolved extract by a pore electrical resistance method is effective in guaranteeing the size of the oxide inclusion.

It has further become apparent that both corrosion resistance and rolling fatigue life can be improved when intermediate annealing and secondary quenching/tempering are performed successively after carburizing treatment.

That is, in the invention, after steel containing oxide inclusions each having a maximum diameter of not larger than 50 is carburized, the steel is subjected to intermediate annealing and secondary quenching/tempering successively so that the steel exhibits a surface C concentration of not lower than 0.9%, contains carbide having an area percentage of not higher than 15 % and contains 0.1 % by area or less rod-like carbide having an aspect ratio of not lower than 3 and having a minor diameter of not smaller than 2 µm.

In the invention, the steel may further contain 0.05 wt% to 1.0 wt% of V, and 0.1 wt% or less of Nb as alloy components.

When these components are contained in the steel, crystal grains can be made so fine that characteristic of the bearing steel can be improved.

The reason why each of the chemical components in the invention is limited will be described below in detail.

### C: 0.10 % to 0.35 %

The amount of C needs to be not smaller than 0.10 % in order to obtain required strength as bearing steel and keep sufficient surface hardness after carburizing treatment. If the content of C is larger than 0.35 %, both toughness and machinability are reduced. Accordingly, the content of C is selected to be in a range of from 0.10 % to 0.35 %.

### Si: < 0.5 %

Si is effective in making a quench-hardened martensitic structure dense to thereby improve toughness and fatigue resistance of steel. In this sense, Si is a significant component in the invention. Corrosion resistance of steel, however, deteriorates remarkably if the amount of added Si is not smaller than 0.5 %. Furthermore, both toughness and processability deteriorate. Accordingly, the content of Si is selected to be smaller than 0.5 %.

### Mn: 0.2 % to 1.5 %

Mn is an element which operates as a deacidifying and desulfurizing element at the time of melting steel and which is effective in improving hardenability of steel. In this invention, therefore, the steel contains 0.2 % or more of Mn. Both processability and machinability, however, deteriorate if the content of Mn is larger than 1.5 %. Accordingly, the upper limit of the content of Mn is set at 1.5 %.

### P: ≤ 0.03 %

### S: ≤ 0.03 %

Eachof P and S causes deterioration of strength of bearing steel. In the invention, therefore, the amount of each of P and S is limited to be not larger than 0.03 %.

### Ni: 1.0 % to 3.5 %

Ni is a significant component in the invention and has a great effect on improvement in corrosion resistance of steel. Ni is an element effective in improving hardenability of steel and toughness of steel after quenching/tempering. In the invention, therefore, the steel contains 1.0 % or more of Ni. Both toughness and processability of steel, however, deteriorate if the content of Ni is larger than 3.5 %. Accordingly, the upper limit of the content of Ni is set at 3.5 %. Preferably, the content of Ni is set from 2.0 to 3.0%.

### Cr: 1.0 % to 5.0 %

Cr is also a significant component in the invention and has a great effect on improvement in corrosion resistance of steel. Cr is an element effective in improving hardenability of steel and strength and toughness of steel after quenching/tempering. In the invention, therefore, the steel contains 1.0 % or more of Cr. If the content of Cr is larger than 5.0 %, both hardenability and machinability, however, deteriorate while the effect on improvement in corrosion resistance is saturated. Accordingly, the upper limit of the content of Cr is set at 5.0 %. Preferably, the content of Cr is set from 1.0 to 2.0 %.

### Mo: 0.03 % to 2.5 %

Mo is an element effective in improving strength of steel. In the invention, therefore, the steel contains 0.03 % or more of Mo. Both hardenability and machinability, however, deteriorate simultaneously if the content of Mo is larger than 2.5 %. Accordingly, the upper limit of the content of Mo is set at 2.5 %. Preferably, the contents of Mo is set from 0.3 to 1.0 %.

### Al: 0.005 % to 0.050 %

Al forms AlN effective in making crystal grains fine. In the invention, therefore, the steel contains 0 .005 % or more of Al. The effect on prevention of production of coarse crystal grains is however reduced as well as cleanliness of steel deteriorates if the content of Al is larger than 0.050 %. Accordingly, the upper limit of the content of Al is set at 0.050 %.

### Ti: ≤ 0.003 %

Ti generates a hard precipitate TiN which operates as a fracture start point of rolling fatigue fracture and which causes reduction in rolling fatigue life. In the invention, therefore, the content of Ti is limited to be not larger than 0.003 %.

### O: ≤ 0.0015 %

O reduces cleanliness of steel to cause reduction in rolling fatigue life. In the invention, therefore, the content of O is limited to be not larger than 0.0015 %.

### N: ≤ 0.025 %

N is bonded to Al to generate AlN which operates to make crystal grains fine. Strength of steel, however, deteriorates if a large amount of N is contained. In the invention, therefore, the upper limit of the content of N is set at 0.025 %. More preferably, the content of N is in a range of from 0.01 % to 0.02 %.

### V: 0.05 % to 1.0 %

### Nb: ≤ 0.1 %

Each of V and Nb is an element that contributes to making crystal grains fine- The effect on making crystal grains fine is reduced if the content of each of V and Nb is too large. Accordingly, when each of V and Nb needs to be added as a selected element, the steel contains 0.05 % to 1.0 % of V, and 0.1 % or less of Nb.

### Surface C Concentration

Surface C concentration after heat treatment is important in order to keep strength of steel. A surface C concentration of not lower than 0.9% is required for obtaining required hardness and rolling fatigue life.

In the case of carburizing processing, when the C concentration increases, the percentage of carbide is increased thereby not only deteriorating resistance of corrosion but also deteriorating both rolling fatigue life and impact resistance.

### Carbide

Fine carbide is required for ensuring rolling fatigue life. If the total area percentage of carbide is higher than 15 %, strength of steel is reduced in reverse.

Particularly, if the alloy elements and the heating treatment condition are inappropriate, rod-like carbide 10 having an aspect ratio of not lower than 3 in terms of the ratio of major diameter to minor diameter and having a minor diameter of not smaller than 2 µm is produced as shown in Fig. 1. If the area percentage of the rod-like carbide 10 produced thus is higher than 0.1 %, both rolling fatigue life and impact resistance are reduced remarkably.

### Oxide Inclusion

The presence of an oxide inclusion reduces rolling fatigue life because the oxide inclusion serves as a start point of rolling fatigue fracture. In addition, the presence of such an oxide inclusion large in size reduces corrosion resistance because the interface between the oxide inclusion and a matrix is preferentially corroded under a corrosive environment.

The maximum diameter of each oxide inclusion is controlled to be not larger than 50 µm in order to obtain bearing steel excellent in corrosion resistance and rolling fatigue life.

### Heat Treatment

When the amount of added alloy elements is large after carburizing, there is the possibility that required surface hardness cannot be obtained because the martensitic transformation point (Ms point) of steel becomes so low that a large amount of residual austenite is produced.

Therefore a secondary quenching/tempering is performed.

In this case, intermediate annealing is performed before the second quenching so that the form of carbide is made appropriate to improve hardenability of the matrix. Further, addition of nitrogen is effective in improving corrosion resistance.

### EMBODIMENT

An embodiment according to the invention will be described below in detail.

### <Material>

In a vacuum induction melting furnace, 150 g of steel having chemical components shown in Table 1 was melted and hot-forged at 1200°C to produce a round bar having a diameter of 32 mm or 65 mm. After the round bar was normalized at 900°C, the round bar was subjected to spheroidizing treatment as softening treatment at 760°C to prepare a test material.

For evaluation of cleanliness of the material, a size distribution of oxide inclusion particles was measured by an acid dissolution extraction-pore electrical resistance method (method for measuring volume of particles on the basis of change in electrical resistance at the time of passage of the particles through pores) .

A round bar of Φ20 mm was cut out of an R/2 portion of the material. After the round bar was quenched from 850°C, about 30 g of a 1 mm-thick thin plate was cut out of the round bar and subjected to acid dissolution.

Extraction of oxide inclusions by acid dissolution was performed with a solution of sulfuric acid and permanganic acid.

The extracted oxide inclusions were dispersed into 200 cc of an electrolytic solution. A size distribution of particles in 500 µl of the dispersed solution was measured in the condition of an aperture size (pore size) of 100 µm by the Multisizer made by Beckman Coulter, Inc.

Table 1 shows the measured maximum diameter of the oxide inclusions.

In any test material of steel according to the invention, the maximum diameter of the oxide inclusions was not larger than 50 µm.

### <Corrosion Test>

For evaluation of corrosion resistance, a corrosion test was performed in a humid condition and in a crevice corrosion condition.

Specifically, a roughly processed test specimen having a diameter of 20 mm and a length of 36 mm was cut out of each of the materials. The test specimen was carburized at 960°C for 22 hours in a furnace in an atmosphere of 1.2 % carbon potential as a carburizing condition. After quenched from 860°C, the test specimen was intermediately annealed at 660°C for 4 hours, secondarily quenched at 790°C and tempered at 180°C. After a cylindrical surface of the test specimen was then ground-finished, the test specimen was subjected to the corrosion test.

A combined cycle testing machine was used in the corrosion test. The state of corrosion was examined after each test specimen was left at a test temperature of 49°C ± 1°C with 95 % or higher relative humidity for 24 hours.

With respect to crevice corrosion, the test specimen was placed quietly on a V block so that a contact portion between the V block and the test specimen was in the crevice corrosion condition.

### <Measurement of C Concentration>

A center portion of the test specimen was cut with a micro-cutter and ground-finished. Then, a C concentration distribution from a surface layer of the test specimen was measured by an electron probe microanalyser (EPMA) to thereby obtain the surface C concentration.

### <Measurement of Carbide>

Carbide was measured as follows. A center portion of the test specimen was cut with amicro-cutter and ground-finished. Then, the test specimen was corroded by picral so that carbide came out from the test specimen. The carbide was observed in five visual fields by a 5000-power scanning electron microscope (SEM), so that the area percentage of carbide and the major and minor diameters of all carbide particles as shown in Fig. 1 were measured by image analysis.

### <Rolling Fatigue Test>

A thrust type rolling fatigue test was performed in order to examine rolling fatigue strength of bearing parts.

A ring-like test specimen having an outer diameter of 63 mm, an inner diameter of 28.7 mm and a thickness of 9 mm was cut out of each material so that it was used as a roughly processed test specimen.

The test specimen was subjected to carburizing treatment and quenching/tempering treatment as heat treatment.

The carburizing condition was the same as in the corrosion test specimen.

After the heat treatment, one test surface of the test specimen was ground-finished by 0.15 mm and the other test surface of the test specimen was lapped so that the test specimen was used as a thrust type rolling fatigue test specimen.

A thrust type rolling fatigue testing machine was used in the test. The test was performed in the test condition shown in Table 2.

High-speed steel gas atomized powder having a hardness of 750 Hv and having a particle size of 100 µm to 180 µm obtained by classification was used in the test under a contamination environment.

The rolling fatigue life was evaluated on the basis of the number (L₁₀) of cycles in which the probability of accumulated breakage reached 10 % in a Weibull distribution and the number (L₅₀) of cycles in which the probability of accumulated breakage reached 50 % in a Weibull distribution when the test was repeated by 16 cycles in the same test condition.

**Table 2: Rolling Fatigue Life Test Condition**

| Testing Machine | Thrust Type Rolling Fatigue Life Testing Machine |
|---|---|
| Contact Surface Pressure | 5.5 (4.9) GPa |
| Rotational Speed | 1800 rpm |
| Test Temperature | Ordinary Temperature |
| Lubricating | Turbine #68 |
| Dirt Content | No Dirt (0.25 g/l) |

| | |
|---|---|
| Note) Values put in parentheses show a contaminated rolling fatigue test condition. | |

### <Charpy Impact Test>

A Charpy impact test was performed in order to examine toughness of bearing parts.

A roughly processed test specimen which was 12 mm wide, 14 mm high and 55 mm long and in which a notch having a depth of 1.8 mm and a curvature radius of 10 mm was formed in the lengthwise center of the test specimen was cut out of each of the materials.

The test specimen was subjected to carburizing and quenching/tempering treatment as heat treatment.

The carburizing condition was as follows. The test specimen was carburized at 930°C for 4 hours in a furnace in an atmosphere of 1.2 % carbon potential. After quenched from 850°C, the test specimen was intermediately annealed at 660°C for 4 hours, secondarily quenched from 790°C and tempered at 180°C.

After the heat treatment, the test specimen was ground into a test specimen which was 10 mm wide and 10 mm high and in which a notch having a depth of 2 mm and a curvature radius of 10 mm was formed in the test specimen. The test specimen was subjected to the Charpy test.

A Charpy testing machine was used in the test. Energy absorbed at breakage of the test specimen was measured at ordinary temperature.

### <Results>

Table 3 shows test results of the carburized materials.

In steel according to the invention, the surface C concentration was not lower than 0.9 %, the area percentage of carbide was not higher than 15 %, and the area percentage of rod-like carbide was not higher than 0.1 %. The term "rod-like carbide" used herein means carbide having a major diameter/minor diameter ratio (aspect ratio) of not lower than 3 and having a minor diameter of not smaller than 2 µm.

As is obvious from the test results, corrosion resistance of steel according to the invention in both humid condition and crevice corrosion condition is more excellent than that of steel according to Comparative Examples.

It is obvious from results of the rolling fatigue test that the life of steel according to the invention in a detergent oil condition is longer than that of steel according to Comparative Examples. Although the rolling fatigue life of steel in a contamination condition is reduced by at least one figure compared with that in the detergent oil condition, the life of steel according to the invention is still longer than that of steel according to Comparative Examples.

The Charpy impact value of steel according to the invention is greater than that of steel according to Comparative Examples. It is obvious that the steel according to the invention is excellent in crushing strength as bearing parts.

As described above, alloy components are added while balanced according to the invention. In addition, the surface C concentration, the area percentage of carbide and the area percentage of rod-like carbide after carburizing treatment are made appropriate. As a result, there can be provided bearing steel which exhibits excellent corrosion resistance even in the case where the bearing steel is adapted to bearing parts in a rolling machine, a thermal power generator, a hydraulic power generator, etc. and which is excellent in surface fatigue strength and rolling fatigue life.

## Claims

1. Bearing steel excellent in corrosion resistance consisting of:
0.10 wt% to 0.35 wt% of C;
less than 0.5 wt% of Si;
0.2 wt% to 1.5 wt% of Mn;
0.03 wt% or less of P;
0.03 wt% or less of S;
1.0 wt% to 3.5 wt% of Ni;
1.0 wt% to 5.0 wt% of Cr;
0.03 wt% to 2.5 wt% of Mo;
0.005 wt% to 0.050 wt% of Al;
0.003 wt% or less of Ti;
0.0015 wt% or less of O;
0.025 wt% or less of N;
optional at least one of 0.05 wt% to 1.0 wt% of V, and 0.1 wt% or less of Nb as an alloy component; and
a residual part of Fe,
**characterized in**
**that** the bearing steel after heat treatment performed by carburizing followed by quenching, intermediate annealing, secondary quenching and tempering successively has a surface C concentration of not lower than 0.9 %, a total area percentage of carbide of 15 % or less and an area percentage of 0.1 % or less for rod-like carbide having an aspect ratio of not lower than 3 in terms of the ratio of major diameter to minor diameter with a minor diameter of not smaller than 2 µm, wherein a maximum diameter of each oxide inclusion of said bearing steel being not larger than 50 µm before said heat treatment.

2. The bearing steel according to claim 1, **characterized in that** Ni is set from 2.0 wt% to 3.0 wt%.

3. The bearing steel according to claim 1, **characterized in that** Cr is set from 1.0 wt% to 2.0 wt%.

4. The bearing steel according to claim 1, **characterized in that** Mo is set from 0.3 wt% to 1.0 wt%.

5. The bearing steel according to claim 1, **characterized in that** Ni is set from 2.0 wt% to 3.0 wt%, Cr is set from 1.0 wt% to 2.0 wt% and Mo is set from 0.3 wt% to 1.0 wt%.

6. The bearing steel according to claim 1 or 5, **characterized in that** the surface C concentration after heat treatment with carburizing is lower than 1.2%.

## Patentansprüche

1. Lagerstahl mit guter Korrosionsbeständigkeit, der besteht aus:
0,10 Gew.-% bis 0,35 Gew.-% an C;
weniger als 0,5 Gew.-% an Si;
0,2 Gew.-% bis 1,5 Gew.-% an Mn;
0,03 Gew.-% oder weniger an P;
0,03 Gew.-% oder weniger an S;
1,0 Gew.-% bis 3,5 Gew.-% an Ni;
1,0 Gew.-% bis 5,0 Gew.-% an Cr;
0,03 Gew.-% bis 2,5 Gew.-% an Mo;
0,005 Gew.-% bis 0,050 Gew.-% an Al;
0,003 Gew.-% oder weniger an Ti;
0,0015 Gew.-% oder weniger an O;
0,025 Gew.-% oder weniger an N;
optional 0,05 Gew.-% bis 1,0 Gew.-% an V und/oder 0,1 Gew.-% oder weniger an Nb als eine Legierungskomponente; und
dem restlichen Anteil aus Fe,
**dadurch gekennzeichnet, dass**
der Lagerstahl nach einer Wärmebehandlung, die durch Karbonisierung mit anschließendem Abschrecken, Zwischenausglühen, zweitem Abschrecken und nachfolgendem Tempern ausgeführt ist, eine Oberflächen-C-Konzentration von nicht weniger als 0,9 %, einen Gesamtflächenanteil von Carbid von 15 % oder weniger und einen Flächenanteil von 0,1 % oder weniger für stabartiges Carbid mit einem Aspektverhältnis von nicht kleiner als 3 in Bezug auf das Verhältnis von großem Durchmesser zu dem kleinen Durchmesser mit einem kleinen Durchmesser von nicht kleiner als 2 µm hat, wobei ein maximaler Durchmesser jeder Oxidinklusion des Lagerstahls nicht größer als 50 µm vor der Wärmebehandlung ist.

2. Lagerstahl nach Anspruch 1, **dadurch gekennzeichnet, dass** Ni von 2,0 Gew.-% bis 3,0 Gew.-% eingestellt ist.

3. Lagerstahl nach Anspruch 1, **dadurch gekennzeichnet, dass** Cr von 1,0 Gew.-% bis 2,0 Gew.-% eingestellt ist.

4. Lagerstahl nach Anspruch 1, **dadurch gekennzeichnet, dass** Mo von 0,3 Gew.-% bis 1,0 Gew.-% eingestellt ist.

5. Lagerstahl nach Anspruch 1, **dadurch gekennzeichnet, dass** Ni von 2,0 Gew.-% bis 3,0 Gew.-% eingestellt ist, Cr von 1,0 Gew.-% bis 2,0 Gew.-% eingestellt ist und Mo von 0,3 Gew.-% bis 1,0 Gew.-% eingestellt ist.

6. Lagerstahl nach Anspruch 1 oder 5, **dadurch gekennzeichnet, dass** die Oberflächen-C-Konzentration nach der Wärmebehandlung durch Karbonisierung kleiner als 1,2 % ist.

## Revendications

1. Acier pour roulements ayant une excellente résistance à la corrosion constitué de :
0,10 % en poids à 0,35 % en poids de C ;
moins de 0,5 % en poids de Si ;
0,2 % en poids à 1,5 % en poids de Mn ;
0,03 % en poids ou moins de P ;
0,03 % en poids ou moins de S ;
1,0 % en poids à 3,5 % en poids de Ni ;
1,0 % en poids à 5,0 % en poids de Cr ;
0,03 % en poids à 2,5 % en poids de Mo ;
0,005 % en poids à 0,050 % en poids d'Al ;
0,003 % en poids ou moins de Ti ;
0,0015 % en poids ou moins de O ;
0,025 % en poids ou moins de N ;
éventuellement au moins l'un de 0,05 % en poids à 1,0 % en poids de V, et 0,1 % en poids ou moins de Nb en tant que constituant d'alliage ; et
une partie résiduelle de Fe,
**caractérisé en**
**ce que** l'acier pour roulements après traitement thermique effectué par carburisation suivie d'une trempe, d'un recuit intermédiaire, d'une trempe secondaire et d'un revenu successivement a une concentration de C en surface non inférieure à 0,9 %, un pourcentage surfacique total de carbure de 15 % ou moins et un pourcentage surfacique de 0,1 % ou moins pour du carbure de type bâtonnet ayant un rapport d'aspect non inférieur à 3 en termes du rapport du diamètre majeur au diamètre mineur avec un diamètre mineur non inférieur à 2 µm, un diamètre maximal de chaque inclusion d'oxyde dudit acier pour roulements n'étant pas supérieur à 50 µm avant ledit traitement thermique.

2. Acier pour roulements selon la revendication 1, **caractérisé en ce que** Ni est réglé de 2,0 % en poids à 3,0 % en poids.

3. Acier pour roulements selon la revendication 1, **caractérisé en ce que** Cr est réglé de 1,0 % en poids à 2,0 % en poids.

4. Acier pour roulements selon la revendication 1, **caractérisé en ce que** Mo est réglé de 0,3 % en poids à 1,0 % en poids.

5. Acier pour roulements selon la revendication 1, **caractérisé en ce que** Ni est réglé de 2,0 % en poids à 3,0 % en poids, Cr est réglé de 1,0 % en poids à 2,0 % en poids et Mo est réglé de 0,3 % en poids à 1,0 % en poids.

6. Acier pour roulements selon les revendications 1 ou 5, **caractérisé en ce que** la concentration de C en surface après traitement thermique avec carburisation est inférieure à 1,2 %.
